

March 31, 1936.

J. C. MORRELL

**2,035,910**

## METHOD OF TREATING HYDROCARBONS

Filed Nov. 29, 1933



Inventor:  
Jaque C. Morrell  
By Lee J. Gary  
Attorney

## UNITED STATES PATENT OFFICE

2,035,910

## METHOD OF TREATING HYDROCARBONS

Jacque C. Morrell, Chicago, Ill., assignor to Universal Oil Products Company, Chicago, Ill., a corporation of Delaware

Application November 29, 1933, Serial No. 700,231

4 Claims. (Cl. 196—56)

This application is a continuation in part of my application Serial No. 409,433 filed November 25, 1929.

This invention relates to the treatment of mixtures of hydrocarbon and bituminous materials, particularly coals, and also lignite, peat, pitches, grahamite, albertite and others, and more particularly relates to the production from such mixtures of hydrocarbons and bituminous materials of lower boiling hydrocarbons suitable as motor fuels by cracking or thermal decomposition of the hydrocarbons and the bituminous materials, producing at the same time coke, gas, and other valuable by-products.

In carrying out the process of the invention, a mixture of oil and coal or other bituminous material is made preferably by suspending the latter in the oil in a finely divided state and then subjecting the mixture to heat treatment where- 20 by the mixture is brought to the cracking or conversion temperature, thereby producing low boiling products suitable as motor fuels.

The product so produced possesses high antiknock properties as a motor fuel owing to the cracking of the material distilled from the bituminous substances or which are cracked in situ to produce low boiling products suitable as motor fuel and containing a high percentage of aromatic and unsaturated hydrocarbons which are known to possess high antiknock properties.

In one specific embodiment the invention comprises the introduction of oxygen or a gas containing free oxygen or ozone, such as air, or mixtures of gases comprising free oxygen, as well as inert gases such as flue gas, nitrogen, carbon dioxide with air and oxygen or ozone, into the system where the mixture of hydrocarbon oil and bituminous material, for example coal, are undergoing treatment to partially oxidize the mixture, particularly the suspended bituminous material. Preferably the degree of oxidation is such that intermediate compounds are formed, such as organic acids, aldehydes, ketones and alcohols, and in order to assist in the control both of the rate and kind of reaction, I may introduce catalysts such as metals, metallic oxides or salts of metals, for example, calcium, aluminum, zinc, tin, iron, nickel, lead, copper, and others, and their oxides and salts.

In order to illustrate the operation I will refer to the accompanying drawing:

Raw oil comprising a fraction of petroleum, coal tar and the like, admixed with coal or other bituminous materials such as those mentioned, the latter preferably being suspended in the oil

in a finely divided condition, is pumped by means of pump 1 through line 2 and valve 2' into line 3, where it meets the reflux from hot oil pump 4 entering line 3 and is passed into the heating coil 5 located in furnace 6, wherein the mixture is brought to the conversion temperature. A portion of the raw oil may be pumped from pump 7 into line 2 through control valve 3', or it may be pumped through line 7' controlled by valve 7'' into dephlegmator or fractionator 18, where it receives heat from the vapors rising in dephlegmator 18, and the catalyst, where used, may be mixed preferably in a finely divided state with the raw oil passing through pump 7 or with the mixture of the raw oil and bituminous material passed through pump 1.

Air or oxygen, or other gases containing free oxygen, are pumped by means of pump or compressor 8 through line 9 and valve 9' into line 3, passing with the mixture of hydrocarbon oil and bituminous material, which mixture may or may not contain a catalyst, into the heating coil wherein some conversion into lower boiling products and into intermediate oxidation products occurs. The material leaving heating coil 5 passes through vapor line 10 controlled by valve 11 into reaction chamber 12. Any non-vaporized material deposited in this chamber is withdrawn through line 13 controlled by valve 13'. The coke produced as a result of the treatment accumulates in reaction chamber 12 and may be removed by any of the well known means. I may use several reaction chambers to provide for the operation of one while the other is being cleaned out or a third is being prepared for operation. I may also provide for the introduction of air or oxygen, or other gases containing free oxygen, into the reaction chamber through line 14 controlled by valve 14' and the oxygen containing gas may be introduced at various levels in the chamber through valved connections 15. The vapors leaving reaction chamber 12 pass through vapor line 16 controlled by valve 17 and enter dephlegmator 18. The reflux condensate resulting from the condensation of heavier portions of the vapors entering dephlegmator 18 passes through line 18' and valve 4' to hot oil pump 4, the said reflux condensate being then returned to the heating coil 5 for further conversion. It is to be pointed out particularly that the retreatment of the partially oxidized reflux condensate produces a motor fuel product which is superior in antiknock properties to the retreatment of reflux condensate not subjected to the 55

action of a gas containing free oxygen under cracking conditions.

The vapors leaving dephlegmator 18 pass through line 19 controlled by valve 19' into cooler and condenser 20 controlled by valve 20', the liquid products being collected into receiver 21. The gas passes through line 22 controlled by valve 22' and the liquid product is withdrawn through line 23 controlled by valve 24.

As an illustration of the results obtained by the process of my invention, a mixture containing 80 per cent by weight of a 26 A. P. I. gravity topped Mid-Continent crude oil and 20 per cent by weight of a West Virginia bituminous coal when treated at a pressure of approximately 300 pounds per square inch and a temperature of 925° F. using 5 per cent by weight of air will result in the production of approximately 75 per cent of distillate based on the volume of the oil charged containing approximately 75 per cent of motor fuel, making a total of approximately 56 per cent of motor fuel based on the oil charged. The motor fuel produced was equivalent in antiknock value to approximately 35 per cent benzol mixed with a straight-run Pennsylvania gasoline.

The total coke produced from the mixture of coal and oil cited, based on the volume of oil charged, will be approximately 120 pounds per barrel. A substantial percentage of hydrocarbon oxidation products will be present in the distillate, adding to its antiknock properties. The coke produced by the process is of high quality having a calorific value of approximately 14,500 B. t. u.'s per pound and is generally honeycomb in structure.

The gas produced by the process makes a very good fuel of high calorific value and may be utilized for purposes other than fuel.

Other types of hydrocarbon oils may also be employed in admixture with the bituminous coal, for example, crude oils or fractions thereof generally, including asphaltic base crudes such as those from California, Mexico and the like. Coal tars and lignite tars may also be employed as the hydrocarbon component, although it is to be understood that somewhat different products will be obtained when these tars are employed than when petroleum fractions are employed.

Increasing the amount of air or gas containing free oxygen, and suitably regulating the conditions, will permit control of the process to produce substantial yields of select products of partial oxidation such as those hereinbefore referred to, including alcohols, aldehydes, ketones and acids.

The process may be operated at various temperatures and pressures, for example, from 750° F. to 1000° F., more or less, and in general a cracking temperature, and from 50 pounds per square inch pressure up to 1500 pounds per square inch, more or less. Generally speaking, lower temperatures and pressures may be used in the presence of catalysts.

While I have given specific examples of the yields obtained by the process, it may be readily recognized that the results obtained will depend upon the operating conditions which may be varied over a wide range, and the examples given

are for illustrative purposes only and not in a limiting sense.

I claim as my invention:

1. A process for producing antiknock motor fuel which comprises mixing finely divided solid bituminous material with hydrocarbon oil, passing the mixture in a restricted stream through a heating zone and then discharging the same into an enlarged zone, heating the mixture to a gasoline-producing cracking temperature under pressure in the heating zone and effecting substantial cracking thereof into gasoline, introducing to the mixture passing through the heating zone a gas containing free oxygen in sufficient quantity to form condensable partial oxidation products, separating vapors from residue in the enlarged zone, and condensing the vapors evolved from the thus treated mixture.

2. A process for producing antiknock motor fuel which comprises mixing finely divided coal with hydrocarbon oil, passing the mixture in a restricted stream through a heating zone and then discharging the same into an enlarged zone, heating the mixture to a gasoline-producing cracking temperature under pressure in the heating zone and effecting substantial cracking thereof into gasoline, introducing to the mixture passing through the heating zone a gas containing free oxygen in sufficient quantity to form condensable partial oxidation products, separating vapors from residue in the enlarged zone, and condensing the vapors evolved from the thus treated mixture.

3. A process for producing antiknock motor fuel which comprises mixing finely divided coal with hydrocarbon oil, passing the mixture in a restricted stream through a heating zone and then discharging the same into an enlarged zone, heating the mixture to a gasoline-producing cracking temperature under pressure in the heating zone and effecting substantial cracking thereof into gasoline, introducing to the mixture passing through the heating zone a gas containing free oxygen in sufficient quantity to form condensable partial oxidation products, separating vapors from residue in the enlarged zone, fractionating the vapors and returning the reflux condensate produced thereby for further treatment, and condensing the vapors evolved from the thus treated mixture.

4. A process for producing antiknock motor fuel which comprises mixing finely divided solid bituminous material with hydrocarbon oil, passing the mixture in a restricted stream through a heating zone and then discharging the same into an enlarged zone, heating the mixture to a gasoline-producing cracking temperature under pressure in the heating zone and effecting substantial cracking thereof into gasoline, introducing to the mixture during the cracking thereof an oxidizing catalyst and a gas containing free oxygen in sufficient quantity to form condensable partial oxidation products, separating vapors from residue in the enlarged zone, and condensing the vapors evolved from the thus treated mixture.

JACQUE C. MORRELL.